# EUROPEAN PATENT SPECIFICATION

(11) **EP 1 870 172 B1**
(45) Date of publication and mention of the grant of the patent: **06.07.2011**
(21) Application number: 06722170.5
(22) Date of filing: 27.03.2006
(51) Int. Cl.: B21B 1/46, B21B 13/22, B22D 11/041, B21B 45/08, B22D 11/12

(54) **A CONTINUOUS CASTING AND ROLLING METHOD FOR MEDIUM PLATE**
STRANGGUSS- UND WALZVERFAHREN FÜR MEDIUMPLATTE
PROCEDE DE COULAGE ET DE LAMINAGE EN CONTINU D'UNE TOLE MOYENNE

(30) Priority: 28.03.2005 CN 200510046133
(43) Date of publication of application: 26.12.2007
(73) Proprietor: Angang Steel Company Limited, Liaoning 114003 (CN)
(72) Inventor: LIU, Jie, Anshan, Liaoning 114021 (CN); HUANG, Hao Dong, Anshan, Liaoning 114021 (CN); LI, Long Zhen, Anshan, Liaoning 114021 (CN); YANG, Xu, Anshan, Liaoning 114021 (CN); ZHANG, Leng, Anshan, Liaoning 114021 (CN); MA, Yong Gang, Anshan, Liaoning 114021 (CN); SHA, Xiao Chun, Anshan, Liaoning 114021 (CN); SUN, Yi Kang, Anshan, Liaoning 114021 (CN); WANG, Ming Ren, Anshan, Liaoning 114021 (CN); NA, Jie Fu, Anshan, Liaoning 114021 (CN); ZHANG, Heng Lu, Anshan, Liaoning 114021 (CN); JIN, Fu Xing, Anshan, Liaoning 114021 (CN)
(74) Representative: Tomlinson, Kerry John
(86) International application number: PCT/CN2006/000518
(87) International publication number: WO 2006/102835

(56) References cited:
- CN-A- 1 483 521
- CN-A- 1 483 528
- JP-A- 09 192 705
- JP-A- 2001 353 564
- US-A- 5 191 924
- US-A- 5 430 930
- US-A- 5 564 178
- US-A- 5 634 257
- US-A- 5 991 991

## Description

### Field of the invention

The application belongs to metallurgical metal processing field, more specifically relates to a continuous casting and rolling process for medium plate.

### Description of the related art

Now, the producing technique of continuous hot rolling plate is mainly divided into traditional process and CSP process. The traditional process comprise continuous casting thick billet with thickness of 200mm∼250mm, flame cutting, heating by walking-beam furnace, descaling, rolling by rough rolling group, shearing, descaling, rolling by finishing rolling train, stream cooling, coiling. Although this process has advantages of full categories, high output, flexible production organization and high reduction ratio and so on, this process still has many disadvantages such as heavy casting device, long rolling line, high workshop, large space requirement, large device investment, large billet storeroom, high energy consuming and so on. The CSP process comprises continuous casting thin billet with thickness of 50mm∼70mm, flame cutting, heating by tunnel furnace, descaling, rolling by finishing rolling train, stream cooling, coiling. Although this process has advantages of lowering investment and production cost, omitting rough rolling train, strengthening finishing rolling train, strengthening reduction capability and so on, this process has many disadvantages such as high casting speed, high breakout ratio, too much restriction to production kinds, difficult developing new grades, high investment of tunnel furnace, complicated devices, hard to operate and maintain, rigid production organization, huge cost of accident treatment, low output and so on. Chinese Patent No. 02132970.2 of the same applicant disclosed a continuous casting and rolling process for medium/thin plate (ASP process). The ASP process comprises converter steel-making, continuous casting thick billet with thickness of 100mm∼150mm, flame cutting, heating by walking-beam furnace, descaling, rough rolling by 3+1 rolling train, hot coil box, shearing, descaling, rolling by finishing rolling train, stream cooling, coiling. The ASP process has advantages of low cost, low investment, flexible production organization, simple maintaining, and low accident rate. But it still has disadvantages, for example, it uses too many old devices, the power of the motor of finishing rolling train is low, the speed of the roller table is low, the capacity of water supply is not enough, the strength of rolling mills' transmission system is not enough, the configuration of the power supply system is aging and so on. Therefore, the development of the technology is more or less limited, resulting that output can't reach requirement and the production development also be limited, and further the width precision, surface quality and shape control have certain limitation.

As a related art, US5,991,991 discloses a machine for producing hot-rolled steel strip from input stock of continuously cast strip in sequential work steps, comprising: means for dividing the solidified input stock into initial strip lengths; first means for descaling the surface of the strip lengths; an equalizing furnace arranged downstream of the descaling means, for heating the strip to a rolling temperature; a roughing train having at least two roll passes arranged downstream of the equalizing furnace for roughing the heated strip; coiling and uncoiling stations arranged downstream of the roughing train for intermediately storing the strip; a second, downstream descaling means for descaling the strip leaving the uncoiling stations; a finishing train arranged downstream of the second descaling means for rolling the strip to a finished strip thickness; a continuous casting machine including a cast-rolling device for producing the strip from the input stock at a continuous casting speed of 4 to 8 m/min and a solidification thickness of 90 to 125 mm; and a cooling and insulating line provided between the continuous casting machine and the equalizing furnace, the equalizing furnace having a length of approximately 45 m a width of approximately 5 to 20 m and being arranged downstream of the dividing means and upstream of the roughing train.

### Summary of the invention

The invention is aimed at eliminating the disadvantages of the above plate production process. The objects of the invention is to enhancing some crucial technique so as to save energy, not only improving the heating quality of billet but also improving the uniformity of plate thickness and quality of plate shape. The invention has advantage of high width precision, improves the work rate and output of the rolling mill, and makes the continuous casting and rolling process for medium plate meet the requirement of modem manufacturing.

The production process of the invention substantially employs that of 02132970.2, and also makes some improvements basing on the former process, so as to improve the production capacity of the invention, broaden the range of the production categories, and meanwhile gain new revolution in the fields of shape control, width precision control and surface quality control. The invention also can realize direct rolling of some steel grades.

To achieve the above objects, the solution of the invention is a continuous casting and rolling process for medium plate comprising the following steps:
continuous casting, during molten steel passing through a mold, to forma continuous casting billet having a section thickness of 100mm-170mm and a width of 900mm-2000mm by hydraulic oscillating, continuously bending and continuously straightening;
direct rolling, hot feeding and hot charging by two continuous casters with four streams and four-streams-merging-one technique, in which each of the two continuous casters' knockout roller tables respectively connects with an entering roller table and an exiting roller table of a heating furnace, achieving rapid hot feeding and hot charging or direct rolling for the continuous casting billet; the continuous casting billet is fed to the entering roller table of the heating furnace through a convey roller table, then fed into a walking-beam furnace by a long-course steel loader of the heating furnace in order to be heated; the exiting roller table of the continuous caster connects with the entering roller table of the heating furnace so that the continuous casting billet is directly fed into the heating furnace by the roller table for hot charging, the hot charging temperature averagely is no less than 700 ; and one exiting roller table of the continuous caster connects with the exiting roller table of the heating furnace;
rough rolling by a rough rolling mill with front and back vertical rollers, in which the maximum single-pass side-pressing amount of the vertical rollers is 50mm, the maximum rolling pressure is 3800kN, and the rolling speed is 0~5.89m/s; when rolling, in each pass, acting of front vertical rollers and opening of back vertical rollers are automatically completed by computer, and the automatic control of width is realized through hydraulic automatic width control (AWC);
finishing rolling using speed-up rolling by a finishing rolling train of F1∼F7 with a maximum speed of 22.8m/s, in which vertical rollers are provided before F1; when the thickness of the intermediate billet is 50mm, the maximum pressing amount is 10mm, and the maximum rolling pressure is 1000kN; F1∼F7 finishing rolling train all are provided with a device for axial shifting and bending working rollers with a maximum axial shifting course of ±200mm and a maximum bending force of 1500kN, so as to improve the control of a plate section's thickness difference and plate shape, and realize free rolling; the maximum speed of the roller table before the finishing rolling train may be up to 5.89m/s; an edge heater is provided before the finishing rolling train;
stream cooling using a three-stage stream cooling technique, in which a roughly adjusting valve set and a precisely adjusting valve set as well as an online high-level water tank are provided, so as to stabilize a water amount and a water pressure of each cooling stage; the side water-jet pressure is 1MPa∼1.2MPa so as to assure the plate's lengthwise temperature uniformity;
coiling with a stepping-controlled full hydraulic coiler, in which automatic stepping control is performed by a hydraulic-controlled side guide, pinch roller, wrapper roller's collapsible reels and high-responsivity wrapper roller to realize precise centering and micro-tension coiling of the plate, reduce towered-shape, avoid the impaction of the plate's head on the wrapper roller and eliminate impression of the plate's head and the wrapper roller on the plate.

In said continuous casting, direct rolling, hot feeding and hot charging, and rough rolling, the exiting roller tables are covered by insulating covers, such that the temperature drop of the casting billet and the temperature difference between the intermediate billet's head and tail are reduced and the temperature of the billet when entering the finishing rolling mill can be increased by 30 °C ∼50°C and the temperature difference between the billet's head and tail can be decreased by 30°C ∼50°C.

In said rough rolling, the vertical roller of the front and back vertical rollers provided in the rough rolling mill is a top-attaching driven type, the size of rollers is φ 1200mm/ φ 1100mm × 430mm, and the power of the main motor is AC1200kW × 2 × 200/400r/min.

In said finishing rolling, the vertical roller of the vertical rollers provided before F1 is a top-driven attached type, the size of rollers is φ 750mm/ φ 600mm × 350mm, and the main drive motor is 2-AC 370kW × 550r/min.

In said finishing rolling, hydraulic low-inertia kinks are provided between the finishing rolling stands in order to control tension between the finishing rolling train and improve plate quality.

In said stream cooling, the cooling device is provided with 12 sets of online high-level water tank with a water amount of 1700m³/h and a water pressure of 0.05MPa∼0.08MPa.

Said mold is a mold for billet continuous casting which has a cavity whose four corners are in the form of a right angle or a round angle or a straight bevel angle, the right angle mold is a traditional billet mold which is composed by two wide sidewalls and two narrow sidewalls with a right angle being formed between respective wide sidewall and narrow sidewall; the round angle or straight bevel angle mold for billet continuous casting is composed by two wide sidewalls and two narrow sidewalls, at both sides of each narrow sidewall, namely the inner sides connected with the wide sidewalls, respectively have a row of right-triangle shaped flange, the bevel of which directs to inside, one right-angle surface joins to the inner surface of the narrow sidewalls, and another right-angle surface is in the same plane with the side face of the narrow sidewalls, namely the another right-angle surface is an extension of the side face of the narrow sidewalls.

By carrying out three kinds of timing control, namely billet merging timing control, billet passing through logistics bottleneck timing control and billet exiting timing control, and comparing cushioning ability, heating ability and rolling ability, said four-streams-merging-one technique optimizes logistics in three walking-beam furnaces with cushioning zone into which the medium plate in single roller table of two casters with four streams is directly fed, so as to exert the producing capacity of caster, furnace and rolling line and realize half-rigid connection of rolling line, furnace and caster.

Said three kinds of timing control are:
Billet converge timing control: which one passes through firstly when two streams from caster A converge; which one passes through firstly when two streams from caster B converge;
   which one passes through firstly when streams from caster A and caster B converge; wherein such principle is followed that when the billets converge, the stream which reaches convergence point firstly passes through firstly and if the two streams reach simultaneously then the straight stream passes through firstly;
Billet passing through logistics bottleneck timing control: determining the timing of No. 1 billet stream charging #1 larry; determining the timing of No. 4 billet stream charging #3 larry; determining the timing of converging No. 1 and No. 2 billet streams charging #2 larry; determining the timing when the billet charging #1 furnace exits A₁ roller table; determining the timing of the billet entering the furnace, wherein such principle is followed that when the billets converge, the stream which reaches convergence point firstly passes through firstly and if the two streams reach simultaneously then the straight stream passes through firstly;
Billet exiting timing control: by tandem superimpose-calculating billet's values at each critical timing as well as checking the cushion capacity and heating capacity of the furnace and
the rolling capacity of the rolling line, finding out billet's values at each critical timing of each condition, realizing semi-rigid connection of caster, furnace and rolling line, wherein such principle is followed that "when the billets converge that the stream which reaches convergence point firstly passes through firstly and if the two streams reach simultaneously then the straight stream passes through firstly".

Compared with prior arts, the invention has the following advantages:
1. Since new mold is used in the present invention, the corner cooling during molten steel solidifying into billet shell in the mold is adjusted from two-dimensional cooling to nearly one-dimensional cooling, so as to make billet shell solidification relatively uniform to avoid surface defect caused by nonuniform
   billet corner's cooling solidification and crack caused by too low edge temperature while direct rolling.
2. The long-course steel loader used in the present invention not only makes the furnace having the ability of heating billet but also has the cushion ability for matching continuous casting and rolling pace. If the rolling mill temporarily halts for a short while, it at most can store nine cushioning billets, therefore the casting production is not affected.
3. The device for axial shifting and bending working rollers provided in all finishing rolling trains not only can control thickness difference of plate section (crown and wedge) and plate flatness, but also can realize free rolling so as to increase rolling yield. The hydraulic low-inertia kinks used in the production line helps to control tension between finishing rolling train and improve plate quality. The speed-up rolling technique used in the finishing rolling trains shortens the feeding time of roller table, reduces temperature drop, improves thickness uniformity and shape quality and increase mill yield and output.
4. The edge heater helps to improve uniformity of billet temperature, reduce edge crack, improve edge microstructure, and stabilize operation of the finishing rolling mill.
5. The use of three-stage stream cooling control technique and the provision of roughly adjusting valve set and precisely adjusting valve set stabilize water amount and water pressure of each cooling stage and assure the plate's lengthwise temperature uniformity, so as to assure uniformity of the plate's microstructure and overcome the production defect caused by water-supply inefficiency in prior arts.

The invention improves the continuous casting and rolling process for medium/thin plate in terms of layout, devices and production process, so that the production ability, development of new grades, production quality are improved with the present invention, production capacity reaches 5000,000t per year, width precision within 0∼10mm reaches 98.5%, the adjustment ability for shape control and crown control reaches advanced world standard, control ability of surface quality fully reaches the quality standard requirements of automobile's high grade panel (05), and the proportion of thin plate reaches advanced world standard.

### Description of embodiment

The invention applies to a continuous casting and rolling process for 2150 medium plate.

Molten steel passes through three 250t top-bottom blowing converter, two molten iron desulphurizing and slag skimming station, two LF ladle furnace and one RH-TB vacuum processing device, and before being cast, it may be refined by LF ladle furnace or RH-TB vacuum processing device.

Continuous casting: molten steel passes through mold, to form continuous casting billet having section thickness of 100mm-170mm, width of 900-2000mm and length of 11m∼18m by hydraulic oscillating, continuously bending and continuously straightening, and then the billet is subjected to flame cutting. The billet has a maximum single weight of 38t, the average number of continuously casting furnaces is 30, and the average casting time is 37.3 minute per one furnace. Because of employing the technique of mold hydraulic oscillating, the quality of casting billet can be improved and also the billet surface defect can be eliminated.

Direct rolling, hot feeding and hot charging by two casters with four streams and four-streams-merging-one technique, in which each of the two continuous casters' knockout roller tables respectively connects with entering roller table and exiting roller table of heating furnace, achieving rapid hot feeding and hot charging or direct rolling for continuous casting billet; continuous casting billet is fed to entering roller table of heating furnace through convey roller table, then fed into walking-beam furnace by long-course steel loader of the heating furnace in order to be heated. Furthermore, the invention uses direct rolling technique for some kinds of carbon steel and certain kinds of lower alloy steel. The exiting roller table of the continuous caster connects with the entering roller table of the heating furnace so that the continuous casting billet is directly fed into the heating furnace by the roller table for hot charging. The hot charging temperature averagely is no less than 700°C. One exiting roller table of the continuous caster connects with the exiting roller table of the heating furnace. Upon billet being on connecting roller table, its length is automatically measured and also its temperature is measured by pyrometer, in order that the billet can be centered according the layout and then be heated. A computer is used to optimize the heating control based on the temperature of the billet entering the furnace. The billets are heated to 1150°C∼1250°C in the furnace, carried out of the furnace by the extractor of the furnace, and placed on the exiting roller table. This can not only save energy, but also shorten heating time and improve heating quality of the billet. Some kinds of carbon steel and certain kinds of lower alloy steel, for example silicon steel, may apply "lower temperature exiting" rolling technique, realizing rolling of different steel grades.

The long-course steel loader used in the present invention not only makes the furnace having the ability of heating billet but also has the cushion ability for matching continuous casting and rolling pace. If the rolling mill temporarily halts for a short while, it at most can store nine cushioning billets, therefore the casting production is not affected.

By carrying out three kinds of timing control, namely billet merging timing control, billet passing through logistics bottleneck timing control and billet exiting timing control, and comparing cushioning ability, heating ability and rolling ability, the four-streams-merging-one technique optimizes logistics in three walking-beam furnaces with cushioning zone into which the medium plate in single roller table of two casters with four streams is directly fed, so as to exert the producing capacity of caster, furnace and rolling line and realize half-rigid connection of rolling line, furnace and caster.

Said three kinds of timing control are:
Billet converge timing control: which one passes through firstly when two streams from caster A converge; which one passes through firstly when two streams from caster B converge; which one passes through firstly when streams from caster A and caster B converge; wherein such principle is followed that "when the billets converge that the stream which reaches convergence point firstly passes through firstly and if the two streams reach simultaneously then the straight stream passes through firstly";
Billet passing through logistics bottleneck timing control: determining the timing of No. 1 billet stream charging #1 larry; determining the timing of No. 4 billet stream charging #3 larry; determining the timing of converging No. 1 and No. 2 billet streams charging #2 larry; determining the timing when the billet charging #1 furnace exits A₁ roller table; determining the timing of the billet entering the furnace, wherein such principle is followed that "when the billets converge that the stream which reaches convergence point firstly passes through firstly and if the two streams reach simultaneously then the straight stream passes through firstly";
Billet exiting timing control: by tandem superimpose-calculating billet's values at each critical timing as well as checking the cushion capacity and heating capacity of the furnace and the rolling capacity of the rolling line, finding out billet's values at each critical timing of each condition, realizing semi-rigid connection of caster, furnace and rolling line, wherein such principle is followed that "when the billets converge that the stream which reaches convergence point firstly passes through firstly and if the two streams reach simultaneously then the straight stream passes through firstly".

Rough rolling: the heated or direct rolled billet is conveyed by roller tables and passes through high-pressure water descaling box after the furnace so as to remove scale, and then enters into four-roller reversible rough rolling mill so as to be rolled. The four-roller reversible rough rolling mill has attached front and back vertical rollers with a type of top-attaching driven. The size of rollers is φ 1200/ φ 1100mm × 430mm, the maximum single-pass side-pressing amount is 50mm, the maximum rolling pressure is 3800kN, the rolling speed is 0∼5.89m/s, and the power of main motor is AC 1200kW × 2 × 200/400r/min. when rolling, in each pass, acting of front vertical rollers and opening of back vertical rollers are automatically completed by computer, and the automatic control of width is realized through hydraulic automatic width control (AWC) in which the front vertical rollers carry out odd pass rolling and the back vertical rollers carry out even pass rolling. The maximum side-pressing amount of each pass is 50mm. After being rolled 3-5 passes in the four-roller reversible rough rolling mill, the billet is rolled into intermediate billet with a thickness of 30∼60mum. During being rolled by the four-roller reversible rough rolling mill, high-pressure water before and after the four-roller reversible rough rolling mill are used to descale regenerated scales of the billet. The front and back vertical rollers of the four-roller reversible rough rolling mill are provided with automatic width control system (AWC), its main purpose being to correct error of billet width caused by rolling pressure change and correct the width difference between the billet's head and tail. Width gage and pyrometer are provided after the four-roller reversible rough rolling mill, so as to monitor width and temperature of billet and provide correction data for setting of finishing rolling mill. The four-roller reversible rough rolling mill is also provided with dust removal device.

Insulating cover is provided at the exiting roller table in order to reduce temperature drop of intermediate billet and temperature difference between the billet's head and tail. Intermediate billet is conveyed to truncate scissor via insulating cover so as to truncate its head and tail. Detector is provided in front of the truncate scissor in order to detect the shape of the billet's head, so as to reduce temperature drop of intermediate billet and temperature difference between the billet's head and tail, and also the temperature at the time of entering finishing rolling mill can be improved by 30°C∼50°C and the temperature difference between the billet's head and tail can be shorten by 30°C∼50°C. Therefore, it can realize the optimal truncation of the scissor, in order to reduce truncation loss and increase yield.

Edge heater is provided in front of the scissor. The heater's parameters are as follows: the power of the main motor is 2 × 3000kW, the heating depth is 40mm∼60mm, the heating width is 100mm∼150mm, and the temperature rise is 60 °C∼100°C. This helps to improve temperature uniformity of the billet, reduce edge crack, and improve mischcrystal of edge microstucture. Also this helps to stabilize operation of the finishing rolling mill, and simultaneously this can satisfy the requirement of dual phase steel development.

After being truncated head and tail, the billet enters into the high-pressure water descaling box before finishing rolling mill in order to remove regeneration scale.

Finishing Rolling: billet passes through the small vertical roller device F₁E before finishing rolling mill F₁ so as to be rolled. When thickness of the intermediate billet is 50mm, the maximum pressing amount is 10mm, the maximum rolling pressure is 1000kN, the main driving motor is 2-AC 370kW × 550r/min. Thereafter the billet enters finishing rolling train. Passing through F1∼F7 four-roller finishing rolling train, the billet is rolled into 1.8mm∼25.4mm final plate.

F1∼F7 finishing rolling train all employ a device for axial shifting and bending working roller, the maximum shifting course is ±200mm, and the bending force is 1500kN. (Only F3~F6 in ASP have the device for axial shifting and bending working roller, and bending force only has positive value, no negative value.) This not only can control thickness difference of plate section (crown and wedge) and plate flatness, but also can realize free rolling and increase rolling yield.

The production line uses hydraulic low-inertia kink in order to control tension between finishing rolling train and improve plate quality.

Stream cooling: it uses three-stage stream cooling technique, in which roughly adjusting valve set and precisely adjusting valve set as well as 12 sets of online high-level water tank are provided, so as to stabilize water amount and water pressure of each cooling stage. The water amount is 1700m³/h, the water pressure is 0.05MPa∼0.08MPa, and the side water-jet pressure is 1Mpa∼1.2MPa, so as to assure the plate's lengthwise temperature uniformity.

Coiling: it uses stepping-controlled full hydraulic coiler to coil plate, in which automatic stepping control is performed by hydraulic-controlled side guide, pinch roller, wrapper roller's collapsible reels and high-responsivity wrapper roller to realize precise centering and micro-tension coiling of plate, reduce towered-shape, avoid the impaction of plate's head on wrapper roller and eliminate impression of plate's head and wrapper roller on plate

The automatic system of the production line is three-grade computer control system, the first grade being basic automatic system, the second grade being procedure control computer system and the third grade being production control computer system.

## Claims

1. A continuous casting and rolling process for medium plate comprising the following steps:
continuous casting, during molten steel passing through a mold, to form a continuous casting billet having a section thickness of 100mm-170mm and a width of 900mm-2000mm by hydraulic oscillating, continuously bending and continuously straightening;
direct rolling, hot feeding and hot charging by two continuous casters with four streams and four-streams-merging-one technique, in which each of the two continuous casters' knockout roller tables respectively connects with an entering roller table and an exiting roller table of a heating furnace, achieving rapid hot feeding and hot charging or direct rolling for the continuous casting billet; the continuous casting billet is fed to the entering roller table of the heating furnace through a convey roller table, then fed into a walking-beam furnace by a long-course steel loader of the heating furnace in order to be heated; the exiting roller table of the continuous caster connects with the entering roller table of the heating furnace so that the continuous casting billet is directly fed into the heating furnace by the roller table for hot charging, the hot charging temperature averagely is no less than 700°C; and one exiting roller table of the continuous caster connects with the exiting roller table of the heating furnace;
rough rolling by a rough rolling mill with front and back vertical rollers, in which the maximum single-pass side-pressing amount of the vertical rollers is 50mm, the maximum rolling pressure is 3800kN, and the rolling speed is 0~5.89m/s; when rolling, in each pass, acting of front vertical rollers and opening of back vertical rollers are automatically completed by computer, and the automatic control of width is realized through hydraulic automatic width control (AWC);
finishing rolling using speed-up rolling by a finishing rolling train of F1~F7 with a maximum speed of 22.8m/s, in which vertical rollers are provided before F1; when thickness of the intermediate billet is 50mm, the maximum pressing amount is 10mm, and the maximum rolling pressure is 1000kN; F1~F7 finishing rolling train all are provided with a device for axial shifting and bending working rollers with a maximum axial shifting course of ±200mm and a maximum bending force of 1500kN, so as to improve the control of a plate section's thickness difference and plate shape, and realize free rolling; the maximum speed of the roller table before the finishing rolling train may be up to 5.89m/s; edge heater is provided before the finishing rolling train;
stream cooling using a three-stage stream cooling technique, in which a roughly adjusting valve set and a precisely adjusting valve set as well as an online high-level water tank are provided, so as to stabilize a water amount and a water pressure of each cooling stage; the side water-jet pressure is 1MPa∼1.2mPa so as to assure the plate's s lengthwise temperature uniformity;
coiling with a stepping-controlled full hydraulic coiler, in which automatic stepping control is performed by a hydraulic-controlled side guide, pinch roller, wrapper roller's collapsible reels and high-responsivity wrapper roller to realize precise centering and micro-tension coiling of the plate, reduce towered-shape, avoid the impaction of the plate's head on the wrapper roller and eliminate impression of the plate's head and the wrapper roller on the plate.

2. The continuous casting and rolling process for medium plate as claimed in claim 1, **characterized in that** in said continuous casting, direct rolling, hot feeding and hot charging, and rough rolling, the exiting roller tables are covered by insulating covers, such that the temperature drop of the casting billet and the temperature difference between the intermediate billet's head and tail are reduced and the temperature of the billet when entering the finishing rolling mill can be increased by 30°C∼50°C and the temperature difference between the billet's head and tail can be decreased by 30°C∼50°C.

3. The continuous casting and rolling process for medium plate as claimed in claim 1, **characterized in that** in said rough rolling, the vertical roller of the front and back vertical rollers provided in the rough rolling mill is a top-attaching driven type, the size of rollers is ϕ1200mm/ϕ1100mm×430mm, and the power of main motor is AC1200kW×2×200/400r/min.

4. The continuous casting and rolling process for medium plate as claimed in claim 1, **characterized in that** in said finishing rolling, the vertical roller of the vertical rollers provided before F 1 is top-driven attached type, the size of rollers is ϕ750mm/ϕ600mm×350mm, and the main drive motor is 2-AC 370kW×550r/min.

5. The continuous casting and rolling process for medium plate as claimed in claim 1, **characterized in that** in said finishing rolling, hydraulic low-inertia kinks are provided between the finishing rolling stands in order to control tension between the finishing rolling train and improve plate quality.

6. The continuous casting and rolling process for medium plate as claimed in claim 1, **characterized in that** in said stream cooling, the cooling device is provided with 12 sets of online high-level water tank with a water amount of 1700m3/h and a water pressure of 0.05Mpa∼0.08Mpa.

7. The continuous casting and rolling process for medium plate as claimed in claim 1, **characterized in that** the structure of said mold is as follows:
said mold is a mold for billet continuous casting which has a cavity whose four corners are in the form of a right angle or a round angle or a straight bevel angle, the right angle mold is a traditional billet mold which is composed by two wide sidewalls and two narrow sidewalls with a right angle being formed between respective wide sidewall and narrow sidewall; the round angle or straight bevel angle mold for billet continuous casting is composed by two wide sidewalls and two narrow sidewalls, at both sides of each narrow sidewall, namely the inner sides connected with the wide sidewalls, respectively have a row of right-triangle shaped flange, the bevel of which directs to inside, one right-angle surface joins to the inner surface of the narrow sidewalls, and another right-angle surface is in the same plane with the side face of the narrow sidewalls, namely the another right-angle surface is an extension of the side face of the narrow sidewalls.

8. The continuous casting and rolling process for medium plate as claimed in claim 1, **characterized in that** by carrying out three kinds of timing control, namely billet merging timing control, billet passing through logistics bottleneck timing control and billet exiting timing control, and comparing cushioning ability, heating ability and rolling ability, said four-streams-merging-one technique optimizes logistics in three walking-beam furnaces with cushioning zone into which the medium plate in single roller table of two casters with four streams is directly fed, so as to exert the producing capacity of caster, furnace and rolling line and realize half-rigid connection of rolling line, furnace and caster.

9. The continuous casting and rolling process for medium plate as claimed in claim 8, **characterized in that** said three kinds of timing control are:
billet converge timing control: which one passes through firstly when two streams from caster A converge; which one passes through firstly when two streams from caster B converge; which one passes through firstly when streams from caster A and caster B converge; wherein such principle is followed that when the billets converge, the stream which reaches convergence point firstly passes through firstly and if the two streams reach simultaneously then the straight stream passes through firstly;
billet passing through logistics bottleneck timing control: determining the timing of No. 1 billet stream charging #1 larry; determining the timing of No. 4 billet stream charging #3 larry; determining the timing of converging No. 1 and No. 2 billet streams charging #2 larry; determining the timing when the billet charging #1 furnace exits A1 roller table; determining the timing of the billet entering the furnace, wherein such principle is followed that when the billets converge, the stream which reaches convergence point firstly passes through firstly and if the two streams reach simultaneously then the straight stream passes through firstly;
billet exiting timing control: by tandem superimpose-calculating the billet's values at each critical timing as well as checking the cushion capacity and heating capacity of the furnace and the rolling capacity of the rolling line, finding out the billet's values at each critical timing of each condition, realizing semi-rigid connection of the caster, furnace and rolling line, wherein such principle is followed that when the billets converge, the stream which reaches convergence point firstly passes through firstly and if the two streams reach simultaneously then the straight stream passes through firstly.

## Patentansprüche

1. Ein Strangguss und Walzverfahren für Mittelbleche weist folgende Schritte auf:
Strangguss, bei dem eine Stahlschmelze eine Form durchströmt, so dass ein Strangguss-Strang, der eine Profildicke von 100 mm bis 170 mm und eine Breite von 900 mm bis 2000 mm aufweist, durch hydraulisches Schwingen, fortlaufendes Biegen und fortlaufendes Richten ausgebildet wird;
durch direktes Walzen, heißes Beschicken und heißes Beladen durch zwei Stranggießanlagen mit 4 Strömen und einer 4-Ströme-vereinigt-zu-einem-Technik, bei dem die Stanzvorrichtungsbänder der zwei Stranggießanlagen mit einem Ein- bzw. Auslaufband des Brennofens verbunden sind, wird ein schnelles heißes Beschicken und Beladen oder direktes Walzen des Strangs erreicht; der Strang wird dem Brennofen über ein Einlaufband, der Förderrollenbänder aufweist, zugeführt, außerdem wird er einem Gleitschrittofen über einen langen Stahlförderer des Brennofen zugeführt, um aufgeheizt zu werden; das Auslaufband der Stranggießanlagen ist so mit dem Einlaufband des Brennofens verbunden, dass der Strang direkt dem Brennofen über das Band für die heiße Beladung zugeführt wird, die heiße Beladungstemperatur ist durchschnittlich nicht geringer als 700°C; und ein Auslaufband der Stranggießanlage ist mit dem Auslaufband des Brennofens verbunden;
das Vorwalzen wird durch ein Vorwalzwerk mit vertikalen Front- und Rückwalzen ausgeführt, bei dem das Maximum der einzelnen Seitenpresshöhen der vertikalen Walze 50 mm beträgt, die maximale Presskraft 3800 kN ist und die Pressgeschwindigkeit bei etwa 0 - 5,89 m/s liegt; während des Walzens wird bei jedem Durchlauf die Betätigung der vorderen vertikalen Rollen und das Öffnen der hinteren vertikalen Rollen automatisch von einem Computer ausgeführt, und die automatische Steuerung der Breite wird durch eine hydraulische Automatik-Breitensteuerung (AWC) bewirkt;
Fertigwalzen benutzt Beschleunigungsrollen von einer Fertigwalzstraße F1 bis F7 benutzt mit einer maximalen Geschwindigkeit von etwa 22,8 m/s, in der vor F1 vertikale Rollen vorgesehen sind; wenn die Dicke des Zwischenstrangs 50 mm beträgt, beträgt der maximale Pressweg 10 mm und die maximale Walzkraft beträgt 1000 kN; die Fertigwalzstraße F1 bis F7 verwendet alle ein Mittel zur axialen Verschiebung und Biegung der Arbeitswalzen - die maximale Verschiebungsbahn beträgt ± 200 mm und die maximale Biegekraft beträgt 1500 kN - um eine Steuerung/Kontrolle der Blechdickenunterschiede und der Blechformen zu verbessern und Freilauf zu ermöglichen; die maximale Geschwindigkeit des Walzenbands vor der Fertigwalzstraße kann bis zu 5,89 m/s sein; eine Kantenheizung ist vor der Fertigwalzstraße bereitgestellt;
eine Stromkühlung verwendet eine dreistufige Stromkühlungstechnik, in der eine grobe Justierung des Ventileinsatzes und eine genaue Justierung des Ventileinsatzes sowie ein online Wasserhochbehälter bereitgestellt sind, um die Wassermenge und den Wasserdruck in jeder Kühlungsphase zu stabilisieren; der Seitenwasserstrahl-Druck beträgt etwa 1 MPa bis 1,2 MPa, um sicher zu stellen, dass das Blech in Längsrichtung eine gleichmäßige Temperatur hat;
das Aufrollen geschied durch eine stufenweise, steuerbare, vollhydraulische Haspelanlage, bei der die automatische schrittweise Steuerung durch eine hydraulisch kontrollierte Seitenführung, eine Andruckrolle, klappbare Haspeln der Verpackungswalze und hoch ansprechempfindliche Verpackungswalze ausgeübt wird, um ein genaues Zentrieren und Mikro-Spannungs-Aufwickeln der Bleche zu realisieren, die hochragende Form zu verringern, die Impaktion der Kopfplatte auf die Verpackungswalze zu vermeiden und den Druck der Kopfplatte und der Verpackungswalze auf das Blech zu beseitigen.

2. Der Strangguss und das Walzverfahren für Mittelbleche nach Anspruch 1, **dadurch gekennzeichnet, dass** beim Strangguss, beim Walzverfahren, bei der heißen Beschickung und bei der heißen Aufladung, und beim Vorwalzen die hinausgehenden Rollenbahnen so durch eine isolierende Abdeckung abgedeckt sind, dass der Temperaturabfall des Strangs und die Temperaturdifferenz zwischen dem Strang-Kopf und dem Strang-Ende verringert wird und die Temperatur des Strangs bei Eintritt in das Fertigwalzwerk um 30°C bis 50°C erhöht werden kann und die Temperaturdifferenz zwischen dem Strang-Kopf und dem Strang-Ende um 30°C bis 50°C gesenkt werden kann.

3. Der Strangguss und das Walzverfahren für Mittelbleche nach Anspruch 1, **dadurch gekennzeichnet, dass** beim Vorwalzen die vertikale Rolle der vorderen und hinteren vertikalen Rolle, die im Vorwalzwerk vorgesehen ist, eine von oben angetriebene Bauart aufweist, die Größe der Walzen Ø 1200 mm/ 0 1100 mm x 430 mm ist, und der Hauptantriebsmotors ein AC 1200 kWx2x200/400 r/min ist.

4. Der Strangguss und das Walzverfahren für Mittelbleche nach Anspruch 1, **dadurch gekennzeichnet, dass** beim Fertigwalzen die vertikale Rolle der vertikalen Rollen, die vor F1 vorgesehen ist, eine von oben angetriebene Bauart aufweist, die Größe der Walzen Ø 750 mm/ Ø 600 mm x 350 mm beträgt, und der Hauptantriebsmotor ein 2-AC 370 kWx550 r/min ist.

5. Der Strangguss und das Walzverfahren für Mittelbleche nach Anspruch 1, **dadurch gekennzeichnet, dass** beim Fertigwalzen hydraulisch geringe Trägheitsuntersetzungen zwischen den Fertigwalzgestellen vorgesehen sind, um die Spannung zwischen der Fertigwalzstraße zu steuern und um die Blechqualität zu verbessern.

6. Der Strangguss und das Walzverfahren für Mittelbleche nach Anspruch 1, **dadurch gekennzeichnet, dass** bei der Stromkühlung das Kühlungsmittel mit 12 Sätzen von online-Wasserhochbehältern mit einer Wassermenge von 1700 m³/h und einem Wasserdruck von 0,05 MPa bis 0,08 MPa versehen ist.

7. Der Strangguss und das Walzverfahren für Mittelbleche nach Anspruch 1, **dadurch gekennzeichnet, dass** der Aufbau der Form wie folgt ist:
die Form ist eine Form für den Strangguss Strang welche eine Kavität aufweist, dessen vier Ecken in Form eines rechten Winkels oder eines Rundwinkels oder eines Fasenwinkels ausgebildet sind; die rechtwinklig ausgebildete Form ist eine traditionelle Strangform, die sich aus zwei breiten Seitenwänden und zwei schmalen Seitenwänden, mit einem rechten Winkel, der jeweils zwischen den schmalen und breiten Seitenwänden ausgebildet ist, zusammensetzt; die Rundwinkel- oder die Fasenwinkel-Form für den Strang setzt sich aus zwei breiten Seitenwänden und zwei schmalen Seitenwänden zusammen; beidseitig an jeder schmalen Seitenwand, nämlich die inneren Seiten sind mit den breiten Seitenwänden verbunden, beziehungsweise weisen eine Reihe von aneinander geflanschten rechtwinkligen Dreiecken auf, eine Fase welche nach innen gerichtet ist, eine rechtwinklige Oberfläche ist mit der inneren Oberfläche der kurzen Seitenwände verbunden, und eine andere rechtwinklige Fläche liegt in der selben Ebene mit der Seitenfläche der kurzen Wand, nämlich der anderen rechtwinkligen Oberfläche, die eine Verlängerung der Seitenfläche der kurzen Seitenwand ist.

8. Der Strangguss und das Walzverfahren für Mittelbleche nach Anspruch 1, **gekennzeichnet durch** das Durchführen von drei Arten von Zeitsteuerung, nämlich die, bei der der Strang zusammenläuft, bei der der Strang einen logistischen Engpass durchläuft, und bei der der Strang entnommen wird, und **durch** das Vergleichen von Dämpfungsleistungsfähigkeit, Aufheizleistungsfähigkeit und Walzenleistungsfähigkeit; die 4-Strömevereinigt-zu-einem-Technik optimiert die Logistik zwischen den drei Hubbalkenöfen mit Pufferzone, in welche die Mittelbleche auf einer einzelner Rollenbahn aus zwei Laufrollen mit vier Strömen eingespeist werden, um von der Leistungskraft der Laufrolle, des Hubbalkenofens und der Walzenlinie Gebrauch zu machen und die halb-starre Verbindung von Walzenlinie, Hubbalkenofen und Laufrolle zu realisieren.

9. Der Strangguss und das Walzverfahren für Mittelbleche nach Anspruch 8, **gekennzeichnet durch** die drei folgenden Arten von Zeitsteuerung:
der Strang nähert sich der Zeitsteuerung/-regelung: welcher geht zuerst durch, wenn zwei Ströme von Gießanlage A zusammenlaufen, welcher geht zuerst **durch**, wenn zwei Ströme von Gießanlage B zusammenlaufen, welcher geht zuerst **durch**, wenn zwei Ströme von Gießanlage A und B zusammenlaufen, wobei das Prinzip befolgt wird, dass wenn die Stränge zusammenlaufen, der Abschnitt, der die Zusammenlaufstelle zuerst erreicht, diese auch zuerst passiert und wenn zwei Abschnitte diese Stelle gleichzeitig erreichen, dann durchläuft der geradlinige Strom diesen Punkt als erstes;
Zeitsteuerung/-regelung, bei der der Strang einen logistischen Engpass durchläuft: Bestimmung des Takts des Ladevorgangs des # 1 Wagens mit dem Nr. 1 Strang-Stroms, Bestimmung des Takts des Ladevorgangs des # 3 Wagens mit dem Nr. 4 Strang-Stroms, Bestimmung des Takts des Ladevorgangs des # 2 Wagens beim Zusammenbringen der Nr. 1 und Nr. 2 Strang-Ströme, Bestimmung des Taktes, mit welchem der Strang der die #1 belädt, den Ofen am Walztisch A1 verlässt; Festlegung des Takts des Eintritts des Strangs in den Ofen; wobei das Prinzip befolgt wird, dass wenn die Stränge zusammenlaufen, der Abschnitt, der die Zusammenlaufstelle zuerst erreicht, diese auch zuerst passiert und wenn zwei Abschnitte diese Stelle gleichzeitig erreichen, dann durchläuft der geradlinige Abschnitt diesen Punkt als erstes;
Strang Entnahme-Zeitregelung/-steuerung: **durch** eine hintereinander überlagernde Kalkulation der Strang Werte zu jeder bedenklichen Zeit sowie **durch** Überprüfung der Pufferleistung und der Heizleistung des Ofens und **durch** die Walzleistung der Walzenlinie, werden die Strangwerte zu jeder bedenkliche Zeit in jeder Situation ermittelt, und die halb-starren Verbindungen der Rollen, des Ofens und der Walzenlinie werden erfasst, wobei das Prinzip befolgt wird, dass wenn die Stränge zusammenlaufen, der Abschnitt, der die Zusammenlaufstelle zuerst erreicht, diese auch zuerst passiert und wenn zwei Abschnitte diese Stelle gleichzeitig erreichen, dann durchläuft der geradlinige Abschnitt diesen Punkt als erstes.

## Revendications

1. Procédé de coulée continue et de laminage pour tôle moyenne comprenant les étapes suivantes :
coulée continue, en passant de l'acier en fusion à travers un moule, pour former une billette de coulée continue ayant une épaisseur de section de 100 mm à 170 mm et une largeur de 900 mm à 2000 mm par oscillation hydraulique, flexion continue et dressage continu ;
laminage direct, alimentation à chaud et chargement à chaud par deux machines de coulée continue avec quatre flux et technique de fusion de quatre flux en un, dans lequel chacune des tables à rouleaux à décochage des deux machines de coulée continue est raccordée respectivement à une table à rouleaux d'entrée et une table à rouleaux de sortie d'un four de chauffage, produisant une alimentation à chaud et un chargement à chaud ou un laminage direct rapides pour la billette de coulée continue; la billette de coulée continue est alimentée sur la table à rouleaux d'entrée du four de chauffage par l'intermédiaire d'une table à rouleaux de transport, puis alimentée dans un four à longerons mobiles par un dispositif de chargement d'acier à longue portée du four de chauffage afin d'être chauffée ; la table à rouleaux de sortie de la machine de coulée continue est raccordée à la table à rouleaux d'entrée du four de chauffage de sorte que la billette de coulée continue soit directement alimentée dans le four de chauffage par la table à rouleaux pour chargement à chaud, la température de chargement à chaud est en moyenne de pas moins de 700 °C ; et une table à rouleaux de sortie de la machine de coulée continue est raccordée à la table à rouleaux de sortie du four de chauffage ;
laminage brut par un laminoir brut avec des rouleaux verticaux avant et arrière, dans lequel la quantité de pressage latéral monopasse des rouleaux verticaux est de 50 mm, la pression maximale de laminage est de 3800 kN, et la vitesse de laminage est de 0 à 5,89 m/s ; lors du laminage, à chaque passage, l'action des rouleaux verticaux avant et l'ouverture des rouleaux verticaux arrière sont commandées automatiquement par ordinateur, et la régulation automatique de la largeur est effectuée par la commande de largeur automatique (AWC) hydraulique ;
laminage de finition en utilisant le laminage à accélération à l'aide d'un train de laminoirs de finition F1 à F7 avec une vitesse maximale de 22,8 m/s, dans lequel des rouleaux verticaux sont disposés avant F1 ; lorsque l'épaisseur de la billette intermédiaire est de 50 mm, la quantité maximale de pressage est de 10 mm, et la pression maximale de laminage est de 1000 kN ; les laminoirs du train de laminoirs de finition F1 à F7 sont tous pourvus d'un dispositif pour déplacement axial et de rouleaux de travail de flexion avec une course de déplacement axial de ±200 mm et une force de flexion maximale de 1500 kN, de manière à améliorer le contrôle de la différence d'épaisseur et de la forme de tôle d'une section de tôle, et réaliser un laminage libre ; la vitesse maximale de la table à rouleaux avant le train de laminoirs de finition peut aller jusqu'à 5,89 m/s ; un chauffage périphérique est disposé avant le train de laminoirs de finition ;
refroidissement à jet utilisant une technique de refroidissement à jet à trois étages, dans laquelle un ensemble de vannes de réglage grossier et un ensemble de vannes de réglage fin ainsi qu'un réservoir d'eau à haut niveau en ligne sont disposés, de manière à stabiliser la quantité d'eau et la pression hydraulique de chaque étage de refroidissement ; la pression de jet d'eau latéral est de 1 MPa à 1,2 MPa de manière à assurer l'uniformité de la température longitudinale de la tôle ;
bobinage avec un bobineur hydraulique à contrôle de chute pas-à-pas, dans lequel une commande pas-à-pas automatique est effectuée par un guide latéral à commande hydraulique, des bobines amovibles de presse à rouleaux et un rouleau d'enroulement à haute sensibilité pour réaliser un centrage précis et un bobinage à microtension de la tôle, réduire la forme de tour, éviter l'impact de la tête de tôle sur le rouleau enrouleur et éliminer l'impression de la tête de tôle et du rouleau enrouleur sur la tôle.

2. Procédé de coulée continue et de laminage pour tôle moyenne selon la revendication 1, **caractérisé en ce que** dans lesdits coulée continue, laminage direct, alimentation à chaud et chargement à chaud, et laminage brut, les tables à rouleaux de sortie sont recouverts par des couvercles isolants, de sorte que la diminution de température de la billette de coulée et la différence de température entre la tête et la queue de billette intermédiaire soient réduites et que la température de la billette lorsqu'elle entre dans le laminoir de finition puisse être augmentée de 30 °C à 50 °C et que la différence de température entre la tête et la queue de billette puisse être diminuée de 30 °C à 50 °C.

3. Procédé de coulée continue et de laminage pour tôle moyenne selon la revendication 1, **caractérisé en ce que** dans ledit laminage brut, le rouleau vertical des rouleaux verticaux avant et arrière disposés dans le laminoir brut est du type à entraînement suspendu, la taille des rouleaux est ϕ1200 mm/ϕ 1100 mm x 430 mm, et la puissance du moteur principal est CA 1200 kWx2x200/400r/min.

4. Procédé de coulée continue et de laminage pour tôle moyenne selon la revendication 1, **caractérisé en ce que** dans ledit laminage de finition, le rouleau vertical des rouleaux verticaux disposé avant F1 est du type à entraînement suspendu, la taille des rouleaux est ϕ 750 mm/ϕ 600 mm x 350 mm, et la puissance du moteur d'entraînement est 2-CA 370 kWx550r/min.

5. Procédé de coulée continue et de laminage pour tôle moyenne selon la revendication 1, **caractérisé en ce que** dans ledit laminage de finition, des plis hydrauliques à faible inertie sont disposés entre les supports de laminage de finition afin de réguler la tension entre le train de laminoirs de finition et améliorer la qualité de la tôle.

6. Procédé de coulée continue et de laminage pour tôle moyenne selon la revendication 1, **caractérisé en ce que** dans ledit refroidissement à jet, le dispositif de refroidissement est pourvu de 12 ensembles de réservoir d'eau à haut niveau en ligne avec une quantité d'eau de 1700 m³/h et une pression d'eau de 0,05 Mpa à 0,08 Mpa.

7. Procédé de coulée continue et de laminage pour tôle moyenne selon la revendication 1, **caractérisé en ce que** la structure dudit moule est comme suit:
ledit moule est un moule pour coulée continue de billette qui a une cavité dont les quatre coins sont sous la forme d'un angle droit ou d'un angle arrondi ou d'un angle biseauté droit, le moule à angle droit est un moule à billette conventionnel qui est composé de deux parois latérales larges et deux parois latérales étroites, un angle droit étant formé entre une paroi latérale large et une paroi latérale étroite respectives ; le moule à angle arrondi ou à angle biseauté droit pour la coulée continue de billette est composé de deux parois latérales larges et deux parois latérales étroites, sur les deux côtés de chaque paroi latérale étroite, à savoir les côtés internes raccordés aux parois latérales larges, ont respectivement une rangée de brides en forme de triangle rectangle, dont le biseau est dirigé vers l'intérieur, une surface à angle droit est jointe à la surface interne des parois latérales étroites, et une autre surface à angle droit est dans le même plan que la face latérale des parois latérales étroites, c'est-à-dire que l'autre surface à angle droit est une extension de la face latérale des parois latérales étroites.

8. Procédé de coulée continue et de laminage pour tôle moyenne selon la revendication 1, **caractérisé en ce qu'**en conduisant trois types de commande de temporisation, à savoir une commande de temporisation de fusion de billette, une commande de temporisation de goulot d'étranglement logistique de passage de billette et une commande de temporisation de sortie de billette, et la comparaison de la capacité d'amortissement, la capacité de chauffage et la capacité de laminage, ladite technique de fusion de quatre flux en un optimise la logistique dans trois fours à longerons mobiles avec une zone d'amortissement dans lequel la tôle moyenne dans une table à rouleaux unique de deux machines de coulée avec quatre flux est directement alimentée, de manière à exploiter la capacité de production des machine de coulée, four et ligne de laminage et réaliser un raccordement semi-rigide des ligne de laminage, four et machine de coulée.

9. Procédé de coulée continue et de laminage pour tôle moyenne selon la revendication 8, **caractérisé en ce que** lesdits trois types de commande de temporisation sont:
commande de temporisation de convergence de billette : lequel passe en premier lorsque deux flux depuis la machine de coulée A convergent ; lequel passe en premier lorsque deux flux depuis la machine de coulée B convergent ; lequel passe en premier lorsque deux flux depuis la machine de coulée A et la machine de coulée B convergent ; où un tel principe est appliqué selon lequel lorsque les billettes convergent, dont le flux atteint un point de convergence en premier passe en premier et si les deux flux arrivent simultanément, alors le flux rectiligne passe en premier ;
commande de temporisation de goulot d'étranglement logistique de passage de billette : détermination de la temporisation du chargement de flux de billette n° 1 dans l'enfourneuse n° 1; détermination de la temporisation du chargement de flux de billette n° 4 dans l'enfourneuse n° 3 ; détermination de la temporisation du chargement des flux de billette n° 1 et n° 2 convergents dans l'enfourneuse n° 2 ; détermination du temps auquel le chargement de billette du four n° 1 sort de la table à rouleaux A1 ; détermination de la temporisation de l'entrée de la billette du four, où un tel principe est suivi selon lequel, lorsque les billettes convergent, le flux qui atteint le point de convergence passe en premier et si les deux flux arrivent simultanément, alors le flux rectiligne passe en premier ;
commande de temporisation de sortie de billette: par calcul par superposition en tandem des valeurs de billette à chaque temps critique ainsi qu'en vérifiant la capacité d'amortissement la capacité de chauffage du four et la capacité de laminage de la ligne de laminage, détermination des valeurs de billette à chaque temps critique de chaque condition, réalisation d'un raccordement semi-rigide des machine de coulée, four et ligne de laminage, où un principe est suivi selon lequel, lorsque les billettes convergent, le flux qui atteint le point de convergence passe en premier et si les deux flux arrivent simultanément, alors le flux rectiligne passe en premier.
